

Feb. 9, 1932.

J. KOHLMAYER

1,844,428

METALLURGICAL HEAT TREATING

Filed April 26, 1928



Justus Kohlmeyer, Inventor,  
By *Byrne, Townsend & Brickenstein*,  
Attorneys.

## UNITED STATES PATENT OFFICE

JUSTUS KOHLMAYER, OF BERLIN-CHARLOTTENBURG, GERMANY, ASSIGNOR TO  
AMERICAN LURGI CORPORATION, OF NEW YORK, N. Y., A CORPORATION OF NEW  
YORK

## METALLURGICAL HEAT TREATING

Application filed April 28, 1928, Serial No. 273,117, and in Germany April 28, 1927.

This invention relates to a method for producing metals, especially lead, from ores, condensed smokes and fumes, residues and the like.

5 Ores, condensed fumes and flying dusts, residues and similar raw materials, containing metal or metal compounds are usually molten down in a reducing atmosphere in shaft kilns. Condensed fumes and smokes 10 and similar finely divided materials are generally agglomerated into lumps, before charging them into the kiln. Pure lead ores have for a number of years also been subjected, to a hearth refining process for the 15 direct production of lead, thus avoiding kiln processes. This hearth process however requires manual labor and gives residues still rich in lead.

20 The new method according to the invention, which is simple in operation and leads to good yields of metal, is carried out in a revolving cylinder furnace, provided with an interior round or cornered refractory lining.

25 The accompanying drawings illustrate two types of furnaces which are adapted for carrying out this invention.

Fig. 1 shows diagrammatically one form 30 of suitable apparatus, the furnace being shown in vertical longitudinal section;

Fig. 2 is a modified form of furnace, in which only the charging end is shown, in vertical longitudinal section, and

35 Fig. 3 is an elevation of the charging end of the furnace shown in Fig. 2.

At the front side of the cylindrical furnace A is arranged a burner b for oil, coal dust or gas in such a manner, that the flame enters the interior of the furnace A by the opening a, thus heating the furnace to a temperature necessary for the reduction of lead oxide or the decomposition of lead sulfate. The combustion gases leave the furnace A either at the opposite side by a central opening c or by a canal d with slide valve l at the burner side. In the latter case the opening c is closed by a cover e. The combustion gases are thus forced to pass the interior of the furnace twice. On the way from the burner side to the opposite side of the furnace there burns

a flame under pressure in the furnace. This flame together with noncombusted gases and air heats the wall of the furnace opposite the burner side, is mixed there with the non-combusted gases and air and forced upwards 55 into a zone, in which there is no pressure or draft and where the combustion is completed. The draft produced by the chimney in the canal d is regulated in such a manner, that the zero zone of the gas pressure in the furnace is just above the entrance opening a.

It is very important, that the clear diameter of the cylinder furnace be greater than its clear length; at least however the clear diameter of the furnace must be the same 65 as the clear length, as only thus is it possible to heat the furnace walls to the necessary temperature, namely, light red heat.

When the interior of the furnace has been heated to the necessary temperature, the raw 70 material, from which lead is to be produced, is charged into the furnace by a charging device k arranged at the burner or the opposite front side of the furnace. The charging device k is connected with a condensing chamber i, into which the canal d enters.

In order to be able to charge more material into the furnace, a segment shaped piece f of refractory material is inserted into the opening a of the furnace (Figs. 2 and 3). The joint g between the furnace and the insertion piece f must however be above the level of the liquid metal in the furnace in the zone filled with pasty slag, thus avoiding losses of the liquid material. As long as the slag is 85 doughy its surface is bent inwards during the rotation of the furnace; the slag is thereby pressed away from the rotating part of the cylinder wall, thus avoiding passage of the doughy slag through the joint between 90 the stationary insertion piece and the rotating furnace. This liquid metal produced is drawn off through the tap hole h (Fig. 1).

The burner has to be operated such a time, that also the charged material has taken up 95 the temperature present in the interior of the furnace. Then reducing carbon such as granulated coke, ground coal, charcoal or the like is charged into the furnace by the charging device k. Also liquid oil may be 100

atomized by the burner *b* into the furnace and acts as reducing agent. The reducing material charged into the furnace is then also to be heated to the temperature present in the furnace. They may however also be mixed with the raw material to be treated in the furnace and charged and heated together with the raw material. The furnace may be rotated during the charging operation. If this is not the case rotation of the furnace must however begin as soon as the charging operation of the furnace is completed. At this moment the action of the burner may be decreased as much as possible, as the heat accumulated by the brick lining of the furnace is sufficient to keep the reduction process of the raw material going for a certain time. The canal *d* and all the other open parts of the furnace are to be kept closed as much as possible during the reduction of the lead oxide. When the heat accumulated by the brick lining of the furnace is spent and used and the reduction process is not finished yet, the slide valve *l* of the canal *d* has to be opened and the burner *b* is started carefully again, in order to keep the reduction temperature in the interior of the furnace. This careful heating is necessary, in order to avoid an overheating in the interior of the furnace, which would lead to an undue evaporation of lead oxide due to a greater amount of combustion gases present in the furnace.

The small amounts of lead and lead oxide evaporated during the reduction process are recovered again in the condensing chamber *i* behind the furnace. The condensing chamber *i* may be of any kind such as with bags or electrically operated. From this condensing chamber *i* the condensed product is automatically brought back again into the furnace.

When volatile products of different kind are leaving the furnace during the reduction process they may be recovered and brought back separately into the furnace. The following example may serve to illustrate this separate recovery: A zinc or cadmium or arsenic containing lead oxide is condensed in an electrically operated condensing apparatus. This impure for instance zinc containing lead oxide, named hereinafter the main oxide, is reduced in the revolving furnace to lead, the zinc oxide, named hereinafter the secondary oxide, being volatilized during the reduction process. This zinc oxide is condensed in the same electrically operated condensing chamber and brought back together with fresh main oxide into the revolving furnace. This procedure is repeated so often, until the fresh main oxide is rich in zinc oxide. When this is the case, the volatilized zinc oxide is condensed in a second electrically operated condensing chamber, and brought back into a revolving furnace so often, until zinc oxide free from lead is ob-

tained. By such an alternate and repeated treatment of the main oxide and secondary oxide, pure lead on the one hand and pure zinc oxide, cadmium oxide or arsenic acid on the other hand are obtained.

The new method is of especial importance for working up fine smokes, fumes and dusts condensed in electrically operated gas cleaning or dust condensing chambers, which until now had to be agglomerated into lumps, before charging them together with fluxes into kilns. According to the invention these raw materials may be charged directly from a central condensing chamber into the revolving furnace connected with the condensing chamber. Also the addition of fluxes is not necessary. The lead is directly recovered as metal by a single step operation in the revolving furnace connected with the condensing chamber.

When the lead containing raw materials also contain sulfur as lead sulfate or lead sulfide or both, it is possible to obtain lead without addition of carbon according to the following equations:



Lead sulfate may also be reduced to lead sulfide by addition of carbon. If residues of lead oxide remain in the furnace, carbon has to be added. If however residues of lead sulfide are present in the furnace, the amount of lead oxide necessary for the reaction with the lead sulfide may be produced by blowing air into the furnace. The new method and the device are therefore adapted for recovering all the lead present in any form in the raw material. In any case one has to watch that the furnace does not become too hot, in order to avoid volatilization of too great an amount of lead, although this is always recovered. Too high a temperature in the furnace must also be avoided, in order to prevent the lead compounds from becoming very liquid and from forming silicates with the brick lining of the furnace which would result in the destruction of the lining. The content of the furnace must always have a doughy consistence, thus obtaining a good mixture of the raw material with the carbon and a satisfactory reduction of the lead oxide.

The new method is also suitable for the treatment of raw materials containing other metals than lead. Thus for example the new method may be employed especially for those metallurgical reactions, carried through until now in a very uneconomical manner in flame furnaces or kilns. By the simultaneous mixing and heating of the content of the furnace through the flames and combustion gases from above and the hot walls of the revolving furnace from below the rate of reaction is increased considerably. Thus for

example copper and lead containing mattes, speiss and drosses may be worked up according to the invention.

Also tin oxide and copper oxide may be reduced to the respective metals or an intermediate product such as cuprous oxide according to the invention. Also litharge may be oxidized to red lead according to the invention. Finally the new method is also adapted for separating easily volatile substances or metals from difficultly volatile substances and metals. Thus for instance zinc may be volatilized out from ores or oxide mixtures. Also, mixtures of easily reducible and difficultly reducible metal oxides may be treated, for example, a mixture of lead oxide and zinc oxide, in which case the difficultly reducible zinc oxide requiring a high temperature for reduction is enriched in an unreduced state in the residue in the furnace.

I claim:

1. A method for making lead from lead oxide containing raw materials which consists in heating the raw material together with a solid reducing agent in a revolving furnace, having a clear length not greater than its clear diameter and preheated to reaction temperatures, condensing the volatilized products and bringing them back into the furnace repeatedly, until the desired yield of lead is obtained.

2. Process of separating non-volatile metals from ores, smelter products and similar raw materials which comprises charging the raw material and a reducing agent into a revolving furnace preheated to reaction temperatures the clear diameter of which is at least as great as its clear length, heating the mixture in the furnace while revolving the same to such a temperature that reduction takes place within the charge, and supplying heat necessary for further reduction by means of a flame burning within the furnace in the presence of the charge.

3. Process as claimed in claim 2 wherein the flame is reversed and travels the length of the furnace twice.

4. Process as claimed in claim 2 wherein the volatilized products are recovered.

5. Process as claimed in claim 2 wherein the raw material comprises an oxide of the group consisting of lead oxide, copper oxide and tin oxide.

6. A method for making lead from lead oxide containing raw materials which comprises heating the raw material together with a carbon-containing reducing agent in a revolving furnace, having a clear length not greater than its clear diameter and preheated to reaction temperatures, condensing the volatilized products and bringing them back into the furnace repeatedly, until the desired yield of lead is obtained.

7. A method for making lead from lead oxide containing raw materials which com-

prises heating the raw material together with lead sulfide as reducing agent in a rotating revolving furnace, having a clear length not greater than its clear diameter and preheated to reaction temperatures, condensing the volatilized products and bringing them back into the furnace repeatedly, until the desired yield of lead is obtained.

8. A process for separating non-volatile metals from ores smelter products and similar raw materials which comprises heating the raw material in the presence of a reducing agent to such a temperature that reduction takes place within the charge in a preheated revolving furnace the clear diameter of which is at least as great as its clear length and supplying heat necessary for further reduction by means of a flame burning within the furnace in the presence of the charge.

9. Process as claimed in claim 8 wherein the flame is reversed and travels the length of the furnace twice.

10. Process as claimed in claim 8 wherein the volatilized products are recovered.

In testimony whereof I affix my signature.

JUSTUS KOHLMAYER.

75

80

85

90

95

100

105

110

115

120

125

130